

1

2,833,798

METHOD OF DEGREASING WOOL AND  
RECOVERY OF WOOL GREASEDaniel P. Norman, Ipswich, Mass., assignor to Pacific  
Mills, Lawrence, Mass., a corporation of MassachusettsNo Drawing. Application November 2, 1955  
Serial No. 544,612

7 Claims. (Cl. 260—412.8)

The present invention relates to the scouring of, and recovery of wool grease from, raw wool and more particularly is concerned with a solvent wool-scouring process.

The present invention is in the nature of an improvement on the process of my prior copending application, Serial No. 274,820, now Patent No. 2,723,281, dated November 8, 1955. In accordance with said prior application, the raw wool is scoured with methylene chloride ( $\text{CH}_2\text{Cl}_2$ ), thereby removing both the wool grease and the suint in a single extraction operation and providing a well scoured wool, and without producing waste of objectionably high B. O. D.

An object of the present invention is to improve upon the process of my prior application. A further object is to provide a solvent wool-scouring process wherein both grease and suint are removed in a single operation and which is more efficient than prior processes. A further object is to provide a methylene chloride wool-scouring process which is more rapid and hence less expensive than prior processes.

In accordance with the present invention I have now found that the addition to the scouring bath, either just before or at the same time as the methylene chloride is applied to the wool, of a small amount of water, or, less preferably, of a polar organic liquid which is soluble in methylene chloride, unexpectedly greatly increases the efficiency of the scouring process, particularly with respect to removal of the suint component of the raw wool, without in any way damaging the wool or increasing the yield of undesirable wastes and, therefore, provides an improved process which is less expensive and more rapid than prior solvent degreasing processes.

The following examples are given by way of illustration and disclosure of my invention without the intention of limiting it thereto.

## Example I

Four pounds of a commercial blend of fine Australian wool containing 7.94% suint, 3.35% potassium and 16.25% grease was picked and then treated in a stainless steel drum with a volume of extracting liquid just sufficient to completely immerse it. This extraction liquid consisted of methylene chloride saturated with water, i. e., methylene chloride containing about 0.198% of its weight of water. The wool was slowly agitated in the liquid at room temperature, drained on an open stainless steel screen and a small portion was removed, dried and analyzed. The remaining wool was then again treated in the same manner with a fresh batch of scouring liquid. This procedure was repeated to give a total of four scours. Inasmuch as the suint of wool is composed primarily of organic potassium salts or soaps, the potassium concentration is an excellent measure of the amount of suint present on the wool. Potassium determinations on the wool at the end of each scour gave the following results:

2

| After Scour Number | Percent Solids Extracted | Percent Potassium remaining on the wool (Dry Basis) |
|--------------------|--------------------------|-----------------------------------------------------|
| 1.....             | 14.4                     | 1.6                                                 |
| 2.....             | 0.8                      | 1.0                                                 |
| 3.....             | 0.6                      | 0.8                                                 |
| 4.....             | 0.5                      | 0.5                                                 |

Scouring of identical batches of the same wool in the same manner with dry methylene chloride followed by determination of the remaining potassium gave the following results,

| After Scour Number | Percent Potassium remaining (Dry Basis) |
|--------------------|-----------------------------------------|
| 1.....             | 2.0                                     |
| 2.....             | 1.8                                     |
| 3.....             | 1.3                                     |
| 4.....             | 0.8                                     |

showing that the presence of the water in the methylene chloride brings about a very substantial increase in the rate of removal of the suint salts, 3 extractions being more effective in removing suint than 4 extractions with dry methylene chloride. Since raw grease wool usually contains from 10 to 18% moisture, it is quite unexpected to find that the addition of as little as 0.198% of moisture to the methylene chloride would produce a very substantial increase in the rate of removal of the suint salts.

The same or even better results can be obtained by adding moisture to the wool, thereby increasing the amount of water over the 0.198% maximum possible when water alone is mixed with the methylene chloride. This procedure is illustrated in the following:

## Example II

A batch of fine Australian wool as in Example I was employed, the batch contained 12% intrinsic or inherent moisture. Before each scour water was added to the wool in an amount equal to 10% of the weight of the wool. Each wool scour was performed as in Example I, with water saturated methylene chloride, and under the same conditions and degree of agitation, with the following results:

| After Scour Number | Percent Potassium remaining on the Wool (Dry Basis) |
|--------------------|-----------------------------------------------------|
| 1.....             | 0.95                                                |
| 2.....             | 0.75                                                |
| 3.....             | 0.40                                                |
| 4.....             | 0.35                                                |

Comparison of these figures with those of Example I shows that two extractions on 22% moisture-containing wool are more efficient than 4 extractions with dry methylene chloride on 12% moisture-containing wool, an advantage of the order of 100% gain in efficiency.

I may increase the amount of water retained by the methylene chloride by use of less than 5% of a water solubilizing compound or "hydrotrope," i. e., a material which will increase the solubility of water in methylene chloride. Many such materials are known and I do not wish my invention to be confined to the use of any particular one or ones. The following example illustrates my process employing sodium benzene sulfonate as such a material.

3  
*Example III*

A batch of fine Australian wool as in Example I was scoured with a solution of methylene chloride containing 0.25% of its weight of sodium benzene sulfonate and 10% water on the weight of the wool. After a single extraction it was found that the amount of potassium left on the wool was only 1.0%, thus indicating that the increased water content of the scouring medium made possible by the solubilizing effect of the sodium benzene sulfonate was as effective in removing suint as was the same amount of water when added to the wool. It is much easier, moreover, to add a hydrotrope and water uniformly to the methylene chloride than to add water uniformly to the wool.

Sodium xylene sulfonate may be substituted for the sodium benzene sulfonate in Example III, in the same amount, with equally good results and I do not intend to exclude salts of other alkyl aryl sulfonates, or exclude other classes of surface active agents.

In the claims I employ the term "mixture" to include not only mixtures but also true solutions.

In accordance with the invention, I also may use a mixture of methylene chloride and a polar organic liquid which is soluble in the methylene chloride. Desirably this liquid is one which forms an azeotropic mixture with the methylene chloride as thus the subsequent distillation treatment, to be described, is facilitated. Representative liquids are methyl alcohol, methyl iodide, carbon disulfide, propylene oxide and glycol, which form such azeotropes, and isopropyl alcohol, acetic acid, benzoic acid, and dicyandiamide which do not. Of these I prefer methyl alcohol as its behaviour is most like that of water. As the azeotrope of methylene chloride and methyl alcohol contains 8% methyl alcohol, the scouring bath will contain sufficient methyl alcohol to introduce risk of felting if an efficient degree of agitation is employed. I prefer, therefore, to dilute this azeotrope with methylene chloride to the extent necessary to prevent undesired felting of the wool.

I believe that any polar organic liquid soluble in methylene chloride is suitable for removing the grease and suint from the wool. In practice, however, there are severe limitations set on the liquids which can be used. These limitations are two-fold: first, the compound must meet the practical criteria of not being too expensive, toxic, difficult to recover, or producing high B. O. D. from small amounts that are eliminated with the miscella wash water. Secondly, it must be readily removable from the wool and, more importantly, from the grease. Most wool grease today finds its ultimate use as a refined product (lanolin) for cosmetic use. Any compound which remains in the grease and could be a skin irritant would obviously be unsuitable for use where the grease is to be so used, even though it would have the desired effect in improving the initial wool scouring process.

I have found that the maximum rate of removal of suint salts in my process occurs when the amount of water or polar organic liquid present is adjusted to be between about 20% and 30%, on the weight of the wool, at the start of the scouring operation, and enough such liquid is added during subsequent scours to maintain about 10% thereof on the dry wool basis. Maximum efficiency of scouring of grease wool by my process is achieved at a water content of about 22%. However, efficient scouring can be effected with water, or equivalent liquid, contents up to about 35%. If the content is increased above 35% the efficiency of the scour drops rapidly, so that the gain in efficiency of suint removal following from such greater moisture content is completely offset by a less effective removal of grease.

Also, too much water in the system may result in felting of the wool. Objectionable felting, or at least risk thereof, does not begin to appear, I have found, until the amount of water present is increased to above about

30%, based on the weight of the wool. The absolute efficiency of the scouring operation depends in a great measure on the degree of agitation of the wool in the liquid medium and the efficiency with which the medium is wrung out of the wool. Proper balance of the water, or equivalent liquid, content against the severity of the agitation should be maintained to obtain the greatest over-all efficiency of the process. In practice a range of from 20% to 27% of water represents a very efficient and practical level for scouring. This optimum range can readily be obtained by spraying the wool coming from the picker or opener with a fine mist or by passing steam through it. Due to the fact that the scouring liquor is largely methylene chloride, my process permits active and efficient agitation of the wool in the bath with little if any risk of felting of the wool, while approaching the efficiency of the conventional aqueous scouring system, so far as suint removal is concerned.

The scouring liquor from the procedure of the foregoing examples is prepared for recovery of grease therefrom by washing it with an equal volume of water with violent agitation, preferably employing two washes. The miscellas formed by addition of water to these scouring liquors, surprisingly, do not form stable emulsions but readily break upon standing or centrifugal treatment so that the aqueous layer containing the suint and dirt is readily separated.

Analysis of a typical separated aqueous layer gave the following results:

| From<br>Scour No. | First Washing |                   |          | Second Washing |                   |          |
|-------------------|---------------|-------------------|----------|----------------|-------------------|----------|
|                   | Percent<br>K  | Percent<br>Grease | B. O. D. | Percent<br>K   | Percent<br>Grease | B. O. D. |
| 35                |               |                   |          |                |                   |          |
| 1-----            | 1.1           | 0.18              | 0.41     | 0.29           | 0.04              | 0.61     |
| 2-----            | 0.32          | 0.14              | 0.30     | 0.068          | 0                 | 0.40     |
| 3-----            | 0.18          | 0.03              | 0.06     | 0.067          | 0                 | 0.14     |
| 4-----            | 0.18          | 0.03              | 0        | 0.067          | 0                 | 0        |
| 5-----            | 0.11          | 0.02              | -1.44    | 0.038          | 0                 | -1.44    |
| 40 Totals....     | 1.89          | 0.40              | 0.67     | 0.530          | 0.04              | 0.29     |

As shown by these data, the suint is effectively removed from the scouring liquor by water washing and the B. O. D. (biological oxygen demand) of the wash water is very low per pound of raw wool.

The suint salts may be recovered from the wash water where this is economically practicable, thereby further reducing the B. O. D. of the effluent. It is entirely possible in my process to discharge the waste wash water directly into a stream with little or no pollution problem, a very important advantage.

The water-washed grease-solvent miscella can be readily further processed by the procedures described in my said prior application Serial No. 274,820 to recover a high quality grease therefrom. Briefly, the miscella can be readily filtered and may be further purified by passing it through an absorption column containing, for example, activated carbon, activated silica gel or activated clay for the removal from the grease of organic impurities. If desired the free fatty acids of the grease may be neutralized and the resultant soaps washed out with water.

Finally the solvent will be removed by distillation. Because of the removal of color-forming impurities prior to distillation, which my process permits, the grease is not discolored in the distillation operations, and a final grease product of exceptional quality may readily be produced.

My scouring process is not restricted to any particular type of equipment. The process may be operated as a batch process or, preferably, as a continuous process. Desirably wholly enclosed equipment is employed so that the methylene chloride may be recovered. Suitable equipment available commercially has been described in United States Patent No. 2,368,916, Drum et al., as well as in many older patents, such as No. 899,440, to Shuman.

In one preferred type of apparatus, the methylene

chloride and water is sprayed onto the wool as it moves along a continuous conveyor, the water being sprayed either simultaneously with or immediately preceding the methylene chloride spray.

In one such operation employing counter-current extraction, the moisture on the wool was adjusted to 22% at the start, water-saturated methylene chloride was employed and the ratio of the methylene chloride to the wool was approximately 30 to 1 by weight. It was found that the potassium content was reduced to 0.25% and the grease content to 0.2%, both by weight on the wool. In contrast, dry methylene chloride alone under identical conditions required a ratio of methylene chloride to wool of 280 to 1 to produce the same results. In the operation just described, 10% of water, by weight of the wool was added just before the first scour, subsequent scourings then being performed with water-saturated methylene chloride without addition of further water. This is a very convenient operating compromise which gives a high desuiting rate with a minimum of control difficulties. The desuiting rate can be increased by adding moisture to the wool at intermediate stages to maintain at least 10% moisture on the wool throughout the whole scouring operation.

I claim:

1. The process for the removal of suint and wool grease from raw wool which comprises leaching the raw wool containing wool grease and suint with a mixture of methylene chloride and a liquid selected from the class consisting of water and polar organic liquids soluble in methylene chloride, to extract wool grease and suint therefrom, the amount of said liquid being less than 35% by weight on the wool.

2. The process for the removal of suint and wool grease from raw wool which comprises leaching the raw wool containing wool grease and suint with a mixture of methylene chloride and a liquid selected from the class consisting of water and polar organic liquids soluble in methylene chloride, to extract wool grease and suint therefrom, separating the liquid extract from the wool fibers, washing the extract with water, and separating the aqueous phase containing suint from the non-aqueous phase containing wool grease, the amount of said liquid being less than 35% by weight on the wool.

3. The process for the removal of suint and wool grease from raw wool which comprises leaching the raw wool containing wool grease and suint with a liquid mixture including methylene chloride and water, the amount of

the water being less than 35% by weight on the wool, thereby to extract wool grease and suint from the wool, separating the liquid extract from the wool fibers, washing the extract with water, and separating the aqueous phase containing suint from the non-aqueous phase containing wool grease.

4. The method of claim 3 wherein the amount of water in the mixture of methylene chloride and water is increased by the presence therewith of a hydrotrope as defined herein.

5. The process for the removal of suint and wool grease from raw wool which comprises adding water to the raw wool to bring its water content within the range 20% to 35% water by weight on the wool, leaching the so modified wool with methylene chloride to extract wool grease and suint therefrom, separating the liquid extract from the wool fibers, washing the extract with water, and separating the aqueous phase containing suint from the non-aqueous phase containing wool grease.

20 6. The process for the removal of suint and wool grease from raw wool which comprises adding water to the raw wool containing wool grease and suint to bring its water content to within the range 20% to 35% water by weight on the wool, leaching the so modified wool with a mixture

25 of methylene chloride and water to extract wool grease and suint therefrom, separating the liquid extract from the wool fibers, washing the extract with water, and separating the aqueous phase containing suint from the non-aqueous phase containing wool grease.

30 7. The process for the removal of suint and wool grease from raw wool which comprises leaching the raw wool containing wool grease and suint with an azeotrope of methylene chloride and methyl alcohol, the amount of the alcohol being less than 35% by weight on the wool, thereby to extract wool grease and suint from the wool, separating the liquid extract from the wool fibers, washing the extract with water, and separating the aqueous-alcohol phase containing suint from the non-aqueous-alcohol phase containing wool grease.

40 **References Cited in the file of this patent**

**UNITED STATES PATENTS**

2,629,723 Lundgren et al. Feb. 24, 1953  
2,723,281 Norman Nov. 8, 1955

**OTHER REFERENCES**

Gillespie: Wool Wax, page 24 (1948), Hobart Publishing Co., Inc., Washington 15, D. C.